

## UNITED STATES PATENT OFFICE

CAMILLE DREYFUS, OF NEW YORK, N. Y., AND WILLIAM WHITEHEAD, OF CUMBERLAND, MARYLAND, ASSIGNEES TO CELANESE CORPORATION OF AMERICA, A CORPORATION OF DELAWARE

## TEXTILE MATERIALS AND METHOD OF PREPARING THE SAME

No Drawing.

Application filed April 17, 1930. Serial No. 445,205.

This invention relates to the preparation or treatment of textile materials, such as yarns or filaments made of organic derivatives of cellulose, whereby the same are rendered more amenable to textile operations or have other improved properties.

An object of our invention is to prepare or treat textile materials, particularly yarns or filaments containing cellulose acetate or other organic derivatives of cellulose, by the employment of oils or fatty acids in conjunction with lecithin, whereby the yarns or filaments are rendered more pliable and can therefore be knitted, woven or knotted more readily. Further objects of our invention will appear from the following detailed description.

In many processes of conversion of textile yarns such as twisting, winding, knitting or weaving, it is desirable to apply finishes which soften or lubricate the yarns. The finishes considered most useful for this purpose contain oils, such as olive or castor oil. However when such oils are applied to the 25 yarn, they tend to polymerize and form viscous and gummy bodies upon ageing. We have found that if lecithin is added to such oils, yarns to which the oil and lecithin have been applied, remain soft and not sticky when 30 exposed to the air for long periods of time.

In accordance with our invention, we employ the animal or vegetable oils or the fatty acids derived therefrom in conjunction with lecithin in the preparation or treatment of 35 textile materials particularly those containing cellulose acetate or other organic derivatives of cellulose.

The animal or vegetable oils employed may be any suitable one such as olive oil, castor 40 oil, cocoanut oil, Neatsfoot oil and in general the glycerides of the fatty acids such as oleic acid, palmitic acid or stearic acid. If desired the fatty acids themselves may be employed. In order to prevent such oils or fatty acids 45 from polymerizing or otherwise becoming sticky and thus imparting harshness to the textile material, we add lecithin thereto. The lecithin may be derived from any source such as from soya beans. While it may be used 50 in the pure state, it is preferable to employ

the product in a form containing some of the oils with which it occurs naturally, since pure lecithin tends to oxidize rapidly. The amount of lecithin employed may be any suitable one say from 0.5 to 5% of the weight 55 of the oils or fatty acids employed in the textile process.

In one form of our invention, the vegetable or animal oils or the fatty acids in admixture with the lecithin may be added to the 60 spinning dope or solution from which the yarns, filaments, artificial bristles or straw are spun, and such solution may then be extruded through orifices into an evaporative atmosphere as in dry spinning or into a precipitating bath as in wet spinning.

In another form of our invention the mixture of the oils or fatty acids and the lecithin may be applied to the yarns, filaments or fabrics after their formation. They may be applied either alone or in admixture with other materials as a lubricant or finish. Thus the lubricant or finish may also contain softening agents such as polyhydric alcohols, examples of which are glycol, diethylene glycol or 75 glycerine.

The textile materials to be prepared or treated in accordance with this invention preferably contain organic derivatives of cellulose which may be organic esters of 80 cellulose or cellulose ethers. Examples of such organic esters of cellulose are cellulose acetate, cellulose propionate, cellulose formate and cellulose butyrate, while examples of cellulose ethers are ethyl cellulose, methyl cellulose and benzyl cellulose.

Yarns, artificial straw or filaments when prepared or treated in accordance with this invention have great pliability due to the presence of the animal or vegetable oils or 90 the free fatty acids, as shown by the fact that such yarns may be readily knitted into a fabric containing many stitches per unit length, and artificial bristles, horsehair and straw may be knotted quite tightly and bent 95 quite severely without breaking. Moreover when such yarns are exposed to the air for long periods of time, because of the presence of the lecithin, they retain their softness and pliability and can be readily knitted.

In order further to illustrate our invention, but without being limited thereto, the following specific example is given.

*Example*

5 A finish is prepared as follows:

Olive oil ----- 99 parts by weight  
Lecithin ----- 1 part by weight

10 The above mixture is applied to a yarn consisting wholly of acetone-soluble cellulose acetate filaments, by causing such yarn to pass over wicks, rollers or other furnishing device for applying such mixture, in their transit  
15 from the spinning machine in which they are formed to a winding device. The amount of finish applied is from 1 to 2% of the weight of the yarn.

10 The yarn so treated is quite pliable and  
20 knits well, takes high twists smoothly and generally exhibits improved properties. Moreover even after ageing in the presence of air or for a long period of time the yarn remains soft and free from stickiness.

25 It is to be understood that the foregoing description is given merely by way of illustration and that many variations may be made therein without departing from the spirit of our invention.

30 Having described our invention, what we desire to secure by Letters Patent is:

1. In a process of preparing or treating textile materials containing organic derivatives of cellulose, the step of introducing a  
35 substance selected from the group consisting of fatty acids and their glycerides in association with lecithin.

2. In a process of preparing or treating textile materials containing cellulose acetate,  
40 the step of introducing a substance selected from the group consisting of fatty acids and their glycerides in association with lecithin.

3. In a process of preparing or treating textile materials containing cellulose acetate, the step of introducing olive oil in association with lecithin.

4. Process of improving the properties of filaments or yarns containing organic derivatives of cellulose comprising applying thereto a finish comprising a glyceride of a fatty acid and lecithin.

5. Process of improving the properties of textile materials containing cellulose acetate comprising applying thereto a finish comprising a glyceride of a fatty acid and lecithin.

6. Process of improving the properties of filaments or yarns containing cellulose acetate comprising applying thereto a finish containing olive oil and lecithin.

7. Textile materials comprising filaments of organic derivatives of cellulose containing a glyceride of a fatty acid and lecithin.

8. Textile materials comprising filaments

of cellulose acetate containing a glyceride of a fatty acid and lecithin.

9. Textile materials containing filaments of cellulose acetate containing olive oil and lecithin.

10 In testimony whereof, we have hereunto subscribed our names.

CAMILLE DREYFUS.  
WILLIAM WHITEHEAD.

75

80

85

90

95

100

105

110

115

120

125

130